

Patented Oct. 29, 1946

2,410,377

# UNITED STATES PATENT OFFICE

2,410,377

## BENEFICIATION OF IRON ORES

Robert B. Booth, Springdale, and Earl C. Herkenhoff, Stamford, Conn., assignors to American Cyanamid Company, New York, N. Y., a corporation of Maine

No Drawing. Application June 18, 1943,  
Serial No. 491,384

6 Claims. (Cl. 209—166)

1

This invention relates to an improved method of beneficiating iron ore by froth flotation.

The problem of iron ore beneficiation has been a serious one because of the low unit value of the product and the fact that, while it is not difficult to float various iron minerals, the procedures employed have resulted in insufficient recovery of concentrates sufficiently rich in iron ore to be commercially usable.

According to the present invention we have found that iron ores can be beneficiated by the use of a class of anionic flotation reagents obtained from the sulfonation of petroleum hydrocarbons. The cheapest and in many respects most satisfactory products are the so-called green acids which are the water soluble products obtained by the treatment of various petroleum lubricating oil fractions with sulfuric acid, oleum, chlorosulfonic acid or other sulfonating agents. These materials are in the main mixtures of indeterminate composition, and it is probable that a considerable proportion of the green acid is in the form of hydrocarbon sulfates rather than true sulfonates, that is to say compounds which have the group  $\text{SO}_3\text{H}$  united to a carbon atom. However, it is customary in the industry to refer to these products as petroleum sulfonates of the green acid type, and, therefore, throughout the present specification and claims the term "petroleum sulfonates of the green acid type" will be used in its common meaning above.

The water soluble petroleum sulfonates are used under definite conditions and the present invention is limited to their use under such conditions and does not cover the use of these reagents generally. According to the present invention the ore must be conditioned with the reagent in the presence of a strong acid. The effectiveness of the acid treatment is not apparently dependent on the nature of the acid anion insofar as it does not have a particular depressant effect and almost any strong or fairly strong acid may be used, either inorganic or organic. The limit of effectiveness appears to lie with acids having an ionization constant of about  $10^{-7}$ . Thus carbonic acid gives barely acceptable results while weaker acids such as boric acid are not satisfactory. Sulfuric acid gives excellent results and because of its extremely low cost it is the preferred acid. Certain strongly acid salts appear to have some effect and may be used, although in most cases they are definitely inferior to the use of the acids themselves.

The mechanism whereby the presence of an acid with the water soluble petroleum sulfonates affects the surface of the particles has not as yet been fully determined and the present invention is not intended to be limited to any particular theory of action. It is important to note that a valuable practical advantage of the present invention lies in the fact that the pH of the circuit is not critical so long as the acid used is strong

5 enough. This obviates the necessity of extremely accurate pH control and permits a material saving in operating supervision. Although the pH and the nature of the particular acid is not critical, there will be optimum conditions for each particular acid. Another factor which has not as yet been fully explained is the fact that it is not necessary that the actual froth flotation take place in a circuit which is strongly acid. On the contrary, if iron ore is conditioned with the hydrocarbon sulfonates and a suitable acid, the pH of the flotation circuit may be modified with alkalies such as soda ash, and, in fact, it is even possible to float in a weakly alkaline circuit. The neutralization appears to have but little effect on the flotation of the acid conditioned ore. This permits, with certain ores, operating practically in a circuit which is not strongly acid, an important commercial advantage because strongly acid circuits require corrosion-proof flotation apparatus, whereas if it is possible to neutralize acid conditioned ore prior to flotation only the conditioning equipment need be made acid proof. This equipment not only represents only a fraction of the total plant, but it is in general of a character which lends itself readily to economical corrosion resistant construction, whereas the flotation machines themselves are more difficult to build and expensive if they must withstand strongly acid circuits.

35 Water soluble petroleum sulfonates and acid alone do not appear to give optimum results and we have found that conditioning in the presence of an oil is desirable for best recoveries and grades. It is an advantage of the present invention that the nature of the oil is not particularly critical. Excellent results are obtained with various hydrocarbon products such as various grades of fuel oil or even crude oil. Since these oils are 40 among the cheapest commercially available materials they may be considered as the preferred oils to be used in the process of the present invention. However, other oily materials are effective such as certain fatty acids, mixtures of fatty and resin acids such as talloel, esters of monohydric alcohols and the like. Esters of glycerin, while effective, appear to give results which are in most cases inferior to the other oils and, while their use is not critical, for best results we prefer to use other oils.

45 Conditioning and flotation procedure is not materially changed by the present invention, which is a further practical advantage as no new operating technique need to be learned. It is desirable to condition the ore with the flotation reagents at high solids, for example from 50-70% which is standard practice in many flotation operations, particularly those involving reagents containing relatively insoluble oils such as fuel oil. Thus, the procedure is standard in the flotation of phosphate rock with fatty acids and fuel oil. Well known conditioning equipment

may, therefore, be used and special apparatus is unnecessary except to the extent that the conditioning apparatus at least must be corrosion proof.

It is an advantage of the process of the present invention that it is not highly sensitive to slimes. In common with almost all froth flotation operations slimes are a detriment, but in the process of the present invention desliming need not be carried to completion, and relatively simple and hence economical desliming operations are quite suitable. It is not necessary to deslime to the completeness which is required with froth flotation operations using cationic reagents. The action of the slime appears to be a normal or usual one, that is to say the presence of small amounts of slime increase the amount of reagent needed for best results, and when the amount of the slime becomes large the grade of concentrate suffers. While the exact behaviour of slime in the present process is not completely known, it is reasonable to assume that it is substantially similar to the action in other froth flotation procedures. The lack of sensitiveness to small amounts of slime is of considerable practical value, as the feed preparation need not be so closely controlled and the cost of desliming equipment may be reduced.

It is an important advantage of the process of the present invention that it is applicable to practically all of the ordinary occurring iron minerals and is not restricted to certain particular ores. As in the case of most froth flotation operations, however, results will differ with different ores. It is an advantage, however, that concentrates of acceptable grade may be produced from low grade ore having iron contents of the order of 12 or 13%. It is also an advantage that the process is so highly selective that in many cases concentrates of satisfactory grade are obtainable in a rougher operation. However, with many ores, and particularly with many low grade ores, cleaning is advantageous, and in common with froth flotation experience on other ores the precise flow sheet for best results will vary somewhat from ore to ore and should be chosen in accordance with best ore dressing practice. The lack of criticalness of the present process, however, makes the choice of plant and procedure simple and no operating difficulties are encountered.

The process of the present invention may be carried out in any suitable flotation machine. Where high outputs are needed, particularly with relatively coarse ore, we have found that the use of highly developed flotation machines of the mechanical type such as Fagergren flotation machines are desirable, but the invention is not limited thereto.

Another advantage of the present invention lies

in the fact that it is not peculiarly susceptible to temperature and can be operated with very cold water. This is of real practical advantage because much of the low grade iron ore for which the present invention is suitable lies in the northern part of the United States where low water temperatures are the rule at the beginning and end of the short mining season.

The process of the present invention may be used with water soluble petroleum sulfonates as the only reagent except for the conditioning acid and oil. It is also possible to associate these reagents with other flotation reagents. For example, mixtures of the water-soluble petroleum sulfonates with oil-soluble petroleum sulfonates, such as the so-called mahogany soaps, give excellent results. The use of oil soluble petroleum sulfonates is not claimed per se in the present invention, but forms the subject matter of our co-pending application, Serial No. 481,906, filed April 5, 1943.

The invention will be described in greater detail in conjunction with the following specific examples. In the examples the froth flotation procedure was standardized. All flotation was effected in Fagergren flotation machines operating at normal speeds and with normal air intake. Flotation time was chosen in each case to obtain good results. In every case the conditioning of the ore with water soluble petroleum sulfonate and acid was effected at high solids, usually about 60-65%.

The petroleum sulfonates of the present invention include the products of reaction of sulfuric acid or oleum with various petroleum lubricating oil fractions. They do not, however, include reaction products of the acid with derivatives such as cracking still gases containing ethylene, propylene and similar molecular gaseous olefines, or light unrefined fuel stocks, such as kerosene fractions.

#### Example 1

A low grade Minnesota iron ore, a reject from an iron beneficiation operation, containing iron largely in the form of hematite with a small amount of limonite, having a gangue high in quartz and containing about 15% Fe was deslimed in the conventional manner, and conditioned at 60-65% solids with various combinations of water soluble petroleum sulfonates with and without sulfuric acid. The conditioned ore was then diluted to flotation density, about 22% solids, and subjected to froth flotation with a single cleaning, except in certain cases where no sulfuric acid was used and the rougher concentrate was obviously too small to be worth cleaning. The metallurgical results appear in the following table:

| Source                    | Name                                  | Lbs./ton | Lbs./ton |               | Concentrate, percent Fe |              | pH of tailings |
|---------------------------|---------------------------------------|----------|----------|---------------|-------------------------|--------------|----------------|
|                           |                                       |          | Fuel oil | Sulfuric acid | Assay                   | Distribution |                |
| L. Sonneborn Sons, Inc.   | Sonesal (green acids)                 | 2.18     | None     | None          | 62.55                   | 19.70        | 6.5            |
| Do                        | do                                    | 2.18     | None     | 1.63          | 61.97                   | 43.00        | 2.5            |
| Do                        | do                                    | 2.18     | 0.94     | None          | 60.35                   | 40.01        | 6.5            |
| Do                        | do                                    | 2.18     | 0.51     | 1.63          | 60.33                   | 92.23        | 2.5            |
| Stanco Distributors, Inc. | SP-702                                | 2.18     | None     | None          | 55.08                   | 16.76        | 6.6            |
| Do                        | do                                    | 2.18     | 1.22     | None          | 49.95                   | 23.78        | 6.6            |
| Do                        | do                                    | 2.18     | None     | 1.63          | 55.08                   | 58.28        | 2.8            |
| Do                        | do                                    | 2.18     | 1.22     | 1.63          | 57.53                   | 78.42        | 2.8            |
| Atlantic Refining Co.     | Petroleum sulfonic acids <sup>1</sup> | 3.27     | 3.59     | None          | 59.05                   | 79.61        | 2.6            |
| Do                        | do                                    | 3.27     | 3.59     | 1.63          | 56.83                   | 83.68        | 2.4            |
| Do                        | Ultrawet                              | 2.18     | 3.59     | None          | 46.10                   | 18.63        | 6.5            |
| Do                        | do                                    | 2.18     | 3.59     | 1.63          | 60.57                   | 79.56        | 2.7            |
| du Pont                   | MP-189                                | 2.14     | 5.07     | 1.63          | 60.00                   | 63.54        | 2.6            |

<sup>1</sup> Contained about 88% sulfonic acids, 10% sulfuric acid, and traces of oil.

It will be apparent that both acid and fuel oil are necessary for good results and that water soluble petroleum sulfonates from a wide variety of sources give satisfactory results.

*Example 2*

The ore of Example 1 was treated as there described, except that no fuel oil was used. A sample of green acids was used as the flotation reagent in the proportion of 2.18 lbs. per ton and the amount of acid varied, two tests being made with no acid but with alkali. The metallurgical results appear in the following table:

| Lbs./ton                       |          | Concentrate, per cent Fe |              | Rougher tailing pH |
|--------------------------------|----------|--------------------------|--------------|--------------------|
| H <sub>2</sub> SO <sub>4</sub> | Soda Ash | Assay                    | Distribution |                    |
| 5.45                           | None     | 60.92                    | 47.47        | 2.1                |
| 2.72                           | None     | 61.38                    | 40.02        | 2.4                |
| 1.63                           | None     | 61.97                    | 43.00        | 2.6                |
| 0.54                           | None     | 61.38                    | 56.37        | 3.0                |
| None                           | 0.54     | 62.55                    | 19.70        | 6.5                |
| None                           | None     | 61.62                    | 30.93        | 8.5                |
| None                           | 3.60     | 61.82                    | 10.88        | 10.1               |

It will be apparent that optimum results are obtainable at a pH of about 3 and that when no acid is used the results drop off sharply.

*Example 3*

The ore and procedure were the same as in Example 1, except for the pulp density in conditioning. Two densities were used, 65% solids and 22% solids. In each case the amount of green acids was 2.18 lbs. per ton. 0.51 lb. per ton of 22° Bé. fuel oil was used with 1.63 lbs. per ton of sulfuric acid. The results appear in the following table:

| Concentrate, per cent Fe |              | Tailing           |     | Pulp density per cent solids |           |
|--------------------------|--------------|-------------------|-----|------------------------------|-----------|
| Assay                    | Distribution | Assay per cent Fe | pH  | Conditioning                 | Flotation |
| 60.33                    | 92.28        | 1.05              | 2.5 | 65                           | 22        |
| 50.71                    | 30.65        | 7.45              | 2.5 | 22                           | 22        |

*Example 4*

The procedure of Example 1 was followed using 2.18 lbs. per ton of a water soluble petroleum sulfonate, SP-702, with varying amounts of fuel oil. The metallurgical results appear in the following table:

| Lbs./ton                       |                | Feed assay, per cent Fe |              | Concentrate per cent Fe |              |
|--------------------------------|----------------|-------------------------|--------------|-------------------------|--------------|
| H <sub>2</sub> SO <sub>4</sub> | Fuel oil No. 2 | Assay                   | Distribution | Assay                   | Distribution |
| None                           | 1.22           | 13.07                   | 49.95        | 23.78                   |              |
| 1.63                           | None           | 12.78                   | 55.08        | 58.28                   |              |
| 1.63                           | 0.61           | 12.72                   | 57.07        | 84.88                   |              |
| 1.63                           | 1.22           | 12.62                   | 57.53        | 78.42                   |              |
| 1.63                           | 1.83           | 12.59                   | 58.23        | 74.06                   |              |

It will be apparent that there is an optimum amount of fuel oil, which for this particular ore and petroleum sulfonate was about 0.6 pound.

*Example 5*

Ore of Example 1 was conditioned at high solids with 2.18 lbs. per ton of water soluble petroleum sulfonate, using SP-702 for the first 13 tests and Sonesal (green acids) for all the remainder but the last test. In the last test 2.18 lbs./ton of a

1:1 mixture of SP-702 and Sonesal was used. The amount of sulfuric acid in every case was 1.63 lbs. per ton. In all cases a rougher concentrate was removed and cleaned once. The different tests were made with different oils. The metallurgical results appear in the following table:

| 10                     | Addition reagent |          | Concentrate, percent Fe |              |
|------------------------|------------------|----------|-------------------------|--------------|
|                        | Type             | Lbs./ton | Assay                   | Distribution |
| None                   |                  |          | 55.08                   | 58.28        |
| Oleic acid             |                  | 0.78     | 56.72                   | 90.39        |
| Coconut oil            |                  | 0.55     | 61.62                   | 43.39        |
| Crude oil              |                  | 0.76     | 53.57                   | 92.69        |
| Chlorinated kerosene   |                  | 0.76     | 59.52                   | 81.04        |
| Tallow                 |                  | 0.82     | 57.18                   | 91.50        |
| Cottonseed oil         |                  | 0.27     | 59.87                   | 50.09        |
| Naphthenic acid        |                  | 0.77     | 54.85                   | 75.51        |
| n-Heptaldehyde         |                  | 0.75     | 56.25                   | 70.15        |
| Fuel oil No. 2         |                  | 0.61     | 57.07                   | 84.88        |
| Methyl ester of tallow |                  | 1.00     | 60.45                   | 75.04        |
| Saponified tallow      |                  | 0.82     | 51.00                   | 84.17        |
| Barrett No. 4          |                  | 0.76     | 50.88                   | 71.80        |
| None                   |                  |          | 61.97                   | 43.00        |
| Crude oil              |                  | 0.76     | 59.63                   | 94.07        |
| Lubricating oil (10-W) |                  | 0.80     | 60.68                   | 75.75        |
| Methyl ester of tallow |                  | 0.78     | 59.05                   | 89.85        |
| "Bunker C" fuel oil    |                  | 0.76     | 59.75                   | 93.29        |
| Chlorinated kerosene   |                  | 0.84     | 60.45                   | 86.70        |
| Coconut oil            |                  | 0.55     | 61.38                   | 63.60        |
| n-Heptaldehyde         |                  | 0.71     | 60.33                   | 80.34        |
| Naphthenic acid        |                  | 0.77     | 50.30                   | 92.74        |
| Lauryl mercaptan       |                  | 0.69     | 60.45                   | 77.28        |
| 22° Bé. fuel oil       |                  | 0.51     | 60.33                   | 92.28        |
| Fuel oil No. 2         |                  | 1.22     | 58.23                   | 83.73        |
| Tallow <sup>1</sup>    |                  | 0.82     | 54.50                   | 91.81        |
| Tallow <sup>1</sup>    |                  | 0.82     | 55.78                   | 93.60        |

<sup>1</sup> In this test 2.18 lbs. of a 1:1 mixture of SP-702 and green acid was used.

*Example 6*

The procedure of Example 1 was followed, except no cleaning was conducted, using 0.51 lb. of 22° Bé. fuel oil in all tests, unless otherwise noted, and varying the acid used. The water soluble petroleum sulfonate was Sonesal (green acids). The metallurgical results appear in the following table:

| 45                                        | Acidic material used |           | Concentrate, per cent Fe |              | Tailing pH |
|-------------------------------------------|----------------------|-----------|--------------------------|--------------|------------|
|                                           | Type                 | Lbs./ton  | Assay                    | Distribution |            |
| Hydrochloric acid                         |                      | 1.63      | 51.70                    | 93.84        | 2.3        |
| Nitric acid                               |                      | 1.63      | 53.10                    | 94.50        | 2.8        |
| Hydrofluoric acid                         |                      | 1.63      | 53.92                    | 94.44        | 3.1        |
| Hydrofluosilicic acid (27%-30%)           |                      | 4.30      | 53.80                    | 90.72        | 3.2        |
| Boric acid                                |                      | 5.45      | 54.73                    | 61.80        | 7.3        |
| Sulfamic acid                             |                      | 2.72      | 50.18                    | 91.62        | 2.5        |
| Perchloric acid                           |                      | 2.30      | 48.20                    | 92.89        | 2.7        |
| Phosphoric acid                           |                      | 2.70      | 50.65                    | 90.66        | 2.5        |
| Sulfurous acid                            |                      | 4.00      | 55.20                    | 96.49        | 3.1        |
| Sulfuric acid                             |                      | 1.63      | 53.95                    | 93.68        | 2.5        |
| Carbonic acid                             |                      | Saturated | 45.86                    | 79.41        | 5.7        |
| Chlorine                                  |                      | Saturated | 49.48                    | 89.70        | 2.1        |
| H <sub>2</sub> S                          |                      | Saturated | 49.71                    | 64.54        | 6.0        |
| Hydrobromic acid (1.03 lbs./ton fuel oil) |                      | 1.34      | 41.38                    | 94.82        | 3.7        |
| Weak oil refinery acid <sup>1</sup>       |                      | 5.23      | 51.58                    | 91.20        | 2.1        |
| Formic acid                               |                      | 3.27      | 46.91                    | 96.02        | 3.1        |
| Acetic acid                               |                      | 2.72      | 50.18                    | 95.27        | 4.0        |
| Acrylic acid                              |                      | 3.60      | 43.30                    | 96.12        | 3.7        |
| Oxalic acid                               |                      | 2.72      | 51.23                    | 81.31        | 2.8        |
| Lactic acid                               |                      | 3.27      | 43.88                    | 96.17        | 3.5        |
| Tartaric acid                             |                      | 3.27      | 51.11                    | 95.85        | 3.2        |
| Citric acid                               |                      | 2.72      | 53.92                    | 93.99        | 3.4        |
| Maleic anhydride                          |                      | 3.27      | 44.58                    | 95.54        | 2.8        |
| Tricarballylic acid                       |                      | 3.60      | 45.74                    | 94.76        | 3.7        |
| Benzolic acid                             |                      | 3.27      | 29.53                    | 87.57        | 3.7        |
| Phthalic acid                             |                      | 3.82      | 44.22                    | 89.81        | 3.4        |
| Salicylic acid (1.03 lbs./ton fuel oil)   |                      | 2.73      | 35.83                    | 91.57        | 3.4        |
| D-Toluene sulfonic acid                   |                      | 2.18      | 50.06                    | 95.89        | 3.3        |
| Phenol (1.03 lbs./ton fuel oil)           |                      | 4.36      | 47.06                    | 61.94        | 7.0        |

<sup>1</sup> Contained about 48% H<sub>2</sub>SO<sub>4</sub>.

It will be apparent that all of the stronger acids work satisfactorily and good results are obtained

down to acids having an ionization constant of  $10^{-7}$ . It should be noted that the somewhat lower grade of concentrate is due to the fact that in the above example there was no cleaning, the data being on rougher flotation alone. For this particular ore cleaning is of importance to obtain concentrates of commercial grade.

*Example 7*

The procedure of Example 1 was followed, but acid salts instead of free acids were used. The metallurgical results appear in the following table:

| Green acids<br>used,<br>lbs./ton | Acidic salt used       |          | Lbs./ton<br>22° Bé.<br>fuel oil | Concentrate, per cent<br>Fe |              | Rougher<br>tailing<br>pH |  |
|----------------------------------|------------------------|----------|---------------------------------|-----------------------------|--------------|--------------------------|--|
|                                  | Type                   | Lbs./ton |                                 | Assay                       | Distribution |                          |  |
|                                  |                        |          |                                 |                             |              |                          |  |
| 3.27                             | Potassium bisulfate    | 10.9     | 1.00                            | 55.90                       | 85.07        | 2.2                      |  |
| 2.18                             | Sodium chlorosulfonate | 5.45     | 0.52                            | 59.87                       | 79.39        | 2.6                      |  |

*Example 8*

A sample of the ore of Example 1 was divided into three parts. One portion was not deslimed at all. A second portion was partially deslimed, using ordinary desliming procedures, and the other was deslimed completely. In each case the ore was conditioned at high solids with green acids, sulfuric acid, and 22° Bé. fuel oil, optimum proportions being used for each product. The completely deslimed material was cleaned once and the partially deslimed and undeslimed material was cleaned twice. The metallurgical results appear in the following table, in which the

It will be noted that the presence of slime required an increase in the amounts of reagents for best results, the increase in the amount of fuel oil needed being particularly striking with the undeslimed ore. At the same time it will be noted that excellent grades were obtainable with good recovery for partially deslimed ore as well as for completely deslimed ore, the latter showing only a slight improvement in grade but permitting the use of materially reduced amounts of reagent. In common with usual flotation practice, operation on completely undeslimed ore was much less economical.

*Example 9*

In order to determine the effects of the reagents of the present invention on various iron minerals present in ores, the pure minerals were ground to -100 mesh, +325 mesh and deslimed prior to flotation. They were conditioned with green acids, fuel oil, and sulfuric acid (in each case there was a blank with no acid, except in the case of goethite), and were floated in a laboratory Fagergren flotation machine. As the minerals are pure, the efficiency of flotation is measured by the percent of material floated. The results appear in the following table:

| Mineral                     | Reagents, lbs./ton             |                      |                | pH  | Weight, grams |       |      | Per cent<br>floated |
|-----------------------------|--------------------------------|----------------------|----------------|-----|---------------|-------|------|---------------------|
|                             | H <sub>2</sub> SO <sub>4</sub> | No. 2<br>fuel<br>oil | Green<br>acids |     | Feed          | Float | Tail |                     |
| Magnetite                   | 8.0                            | 0.75                 | 1.0            | 2.5 | 30.6          | 27.1  | 3.5  | 88.6                |
| Do                          | None                           | 0.75                 | 1.0            | 7.1 | 30.5          | 0.7   | 29.8 | 2.3                 |
| Titaniferous mag-<br>netite | 8.0                            | 0.75                 | 1.0            | 2.3 | 30.1          | 24.6  | 5.5  | 81.7                |
| Do                          | None                           | 0.75                 | 1.0            | 6.9 | 30.2          | 1.2   | 29.0 | 4.0                 |
| Limonite                    | 8.0                            | 1.50                 | 5.0            | 2.5 | 33.6          | 32.2  | 1.4  | 95.8                |
| Do                          | None                           | 1.50                 | 5.0            | 6.6 | 32.7          | 14.8  | 17.9 | 45.3                |
| Goethite                    | 8.0                            | 1.50                 | 5.0            | 2.2 | 29.4          | 29.3  | 0.1  | 99.7                |
| Marite                      | 8.0                            | 0.75                 | 1.0            | 2.4 | 29.4          | 27.1  | 2.3  | 92.2                |
| Do                          | None                           | 0.75                 | 1.0            | 6.9 | 29.9          | 1.1   | 28.8 | 3.7                 |
| Hematite                    | 8.0                            | 3.00                 | 5.0            | 2.9 | 30.8          | 20.1  | 10.7 | 65.3                |
| Do                          | None                           | 3.00                 | 5.0            | 6.8 | 30.4          | 1.4   | 29.0 | 4.6                 |
| Siderite                    | 2.0                            | 0.75                 | 1.0            | 3.3 | 31.3          | 30.8  | 0.5  | 98.5                |
| Do                          | None                           | 0.75                 | 1.0            | 6.6 | 30.9          | 20.3  | 10.6 | 65.7                |
| Ilmenite                    | 8.0                            | 0.75                 | 1.0            | 2.1 | 31.7          | 31.5  | 0.2  | 99.4                |
| Do                          | None                           | 0.75                 | 1.0            | 6.4 | 31.3          | 5.7   | 25.6 | 18.2                |

first test is on completely deslimed, the second on partially deslimed, and the third on undeslimed ore:

*Example 10*

An iron ore of Example 1 was conditioned with mixtures of water soluble petroleum sulfonates

| Product         | Per cent<br>weight | Assay          |                    | Per cent<br>Fe distribu-<br>tion | Lbs./ton used  |                                |             |
|-----------------|--------------------|----------------|--------------------|----------------------------------|----------------|--------------------------------|-------------|
|                 |                    | Per cent<br>Fe | Per cent<br>insol. |                                  | Green<br>acids | H <sub>2</sub> SO <sub>4</sub> | Fuel<br>oil |
| Calc. head      | 100.00             | 14.73          | -----              | 100.00                           | -----          | -----                          | -----       |
| Slime           | 8.19               | 28.96          | -----              | 16.10                            | -----          | -----                          | -----       |
| Clean conc.     | 18.33              | 59.34          | 8.40               | 73.82                            | 2.18           | 1.63                           | 0.51        |
| Clean. tail     | 3.80               | 6.62           | -----              | 1.71                             | -----          | -----                          | -----       |
| Rgh. tail       | 69.68              | 1.77           | -----              | 8.37                             | -----          | -----                          | -----       |
| Head            | 100.00             | 14.92          | -----              | 100.00                           | -----          | -----                          | -----       |
| Slime           | 3.42               | 37.94          | -----              | 8.70                             | -----          | -----                          | -----       |
| Clean conc.     | 18.74              | 58.75          | 9.20               | 73.78                            | 2.72           | 2.18                           | 0.76        |
| 2nd clean. tail | 1.13               | 30.02          | -----              | 2.27                             | -----          | -----                          | -----       |
| 1st clean. tail | 3.35               | 10.99          | -----              | 2.47                             | -----          | -----                          | -----       |
| Rgh. tail       | 73.36              | 2.60           | -----              | 12.78                            | -----          | -----                          | -----       |
| Head            | 100.00             | 14.60          | -----              | 100.00                           | -----          | -----                          | -----       |
| Clean. conc.    | 24.87              | 51.77          | 19.20              | 88.18                            | 2.72           | 2.18                           | 5.12        |
| 2nd clean. tail | 3.56               | 16.08          | -----              | 3.92                             | -----          | -----                          | -----       |
| 1st clean. tail | 5.09               | 5.67           | -----              | 1.98                             | -----          | -----                          | -----       |
| Rgh. tail       | 66.48              | 1.30           | -----              | 5.92                             | -----          | -----                          | -----       |

and various types of mahogany soaps or oil soluble petroleum sulfonates. Conditioning was at high solids and in every case 1.63 lbs. per ton of sulfuric acid were used. The amount of green acids was 1.09 lbs. per ton. In all but one of the tests there was no additional fuel oil. The floats are rougher floats only. The metallurgical results appear in the following table:

| Oil soluble sulfonate used                                           | 22° Bé. fuel oil, lbs./ton | Concentrate, per cent Fe |              | Assay | Distribution |
|----------------------------------------------------------------------|----------------------------|--------------------------|--------------|-------|--------------|
|                                                                      |                            | Assay                    | Distribution |       |              |
| 0.98 lb./ton SP-312 (Stanco Distributors, Inc.)                      | None                       | 59.05                    | 83.03        |       |              |
| 0.98 lb./ton Calol sodium sulfonate (Standard Oil Co. of California) | None                       | 53.33                    | 90.83        |       |              |
| 0.98 lb./ton Calol sodium sulfonate                                  | 0.54                       | 53.33                    | 91.36        |       |              |
| 0.84 lb./ton Ultralate No. 2 (Atlantic Refining Co.)                 | None                       | 58.35                    | 84.37        |       |              |

#### Example 11

The procedure of Example 1 was followed but the ore was first deslimed, then scrubbed or polished by agitation in a flotation cell with the air shut off at 25% solids, and then again deslimed to remove secondary slimes. Conditioning was with 1.63 lbs. per ton of sulfuric acid, 1.09 lbs. per ton green acids, and 0.51 lb. per ton 22° Bé. fuel oil. Two cleaning floats were conducted. The metallurgical results appear in the following table:

| Product            | Per cent weight | Per cent Fe | Per cent insol. | Per cent distribution Fe |
|--------------------|-----------------|-------------|-----------------|--------------------------|
| Head               | 100.00          | 14.68       | -----           | 100.00                   |
| Prim. slime        | 6.14            | 35.46       | -----           | 14.83                    |
| Sec. slime         | 2.40            | 40.42       | 6.61            | 40.42                    |
| Clean. conc.       | 17.15           | 60.52       | 6.60            | 70.70                    |
| Comb. clean. tails | 11.49           | 4.85        | 3.79            | 4.07                     |
| Rgh. tail          | 62.82           | 0.95        | -----           | 4.07                     |

The results should be compared with the completely deslimed ore of Example 8. It will be noted that the grade is slightly higher, the recovery almost as good, and the amount of reagent halved. In many cases the saving in reagent obtainable by scrubbing is commercially worthwhile.

#### Example 12

The ore of Example 1 was deslimed, conditioned at 67% solids with 2.18 lbs. per ton green acids, 1.63 lbs. per ton sulfuric acid and 0.51 lb. per ton 22° Bé. fuel oil. The conditioned ore was then diluted to 22% solids and floated in a Fagergren flotation machine. The concentrate was then conditioned at about 6% solids with 2.18 lbs. per ton of soda ash and 1.63 lbs. per ton of quebracho. The conditioned ore was then deslimed and subjected to cationic flotation in a Fagergren flotation cell, using as reagents 0.12 lb. per ton pine oil and 0.22 lb. per ton laurylamine hydro-

chloride. The metallurgical results of the double float appear in the following table:

| 5                              | Product | Percent weight | Percent Fe |              |
|--------------------------------|---------|----------------|------------|--------------|
|                                |         |                | Assay      | Distribution |
| Feed                           |         | 100.00         | 13.40      | 100.00       |
| Anionic flotation tailing      |         | 74.94          | 1.54       | 8.61         |
| Secondary slime                |         | 1.21           | 37.13      | 3.35         |
| Cationic flotation concentrate |         | 12.90          | 38.77      | 37.32        |
| Cationic flotation tailing     |         | 10.95          | 62.06      | 50.72        |

#### Example 13

The procedure of Example 1 was followed, using 2.18 lbs. per ton green acids and 1.63 lbs. per ton sulfuric acid, except in the case of the sixth test of the first table. This sixth test was a blank test and no sulfuric acid was used. The pulp was then diluted to flotation density and varying amounts of alkali were used to neutralize partly or wholly the acidity. Flotation was then effected and the metallurgical results appear in the following tables, in which the first shows various amounts of soda ash, including the blank test, and the second table shows the effect of various types of alkali:

| 30   | Lbs./ton soda ash | Concentrate, per cent Fe |              | Rougher tailing pH |
|------|-------------------|--------------------------|--------------|--------------------|
|      |                   | Assay                    | Distribution |                    |
| None | 60.33             | 92.28                    | 2.5          |                    |
| 0.54 | 57.88             | 88.25                    | 2.7          |                    |
| 1.63 | 57.53             | 90.25                    | 5.9          |                    |
| 2.18 | 59.57             | 88.71                    | 7.1          |                    |
| 3.60 | 58.86             | 86.25                    | 8.0          |                    |
| 3.60 | 61.82             | 10.88                    | 10.1         |                    |

| 40                | Alkali used |          | Concentrate per cent Fe |              | Rougher tailing pH |
|-------------------|-------------|----------|-------------------------|--------------|--------------------|
|                   | Type        | Lbs./ton | Assay                   | Distribution |                    |
| Calcium carbonate |             | 1.0      | 56.28                   | 87.64        | 3.5                |
| Hydrated lime     |             | 1.0      | 57.94                   | 87.06        | 6.8                |
| Caustic soda      |             | 1.0      | 59.00                   | 86.61        | 6.3                |
| Ammonia           |             | 0.83     | 56.76                   | 87.03        | 8.6                |

It will be apparent that there is but little loss in efficiency when the acid conditioned material is neutralized with alkali.

#### Example 14

The effect of the process of the present invention on various iron ores was tested. In each case the ore was ground, if necessary, deslimed, conditioned at 60-65% solids, diluted to flotation pulp density and floated in a Fagergren flotation machine. Cleaning was effected once, except with the tests marked with an asterisk, where the recleaning was used. In every case the reagent combination giving best results was employed. The metallurgical results appear in the following table:

| Lbs./ton | Source of ore | Feed assay, per cent Fe | Concentrate, per cent Fe |              | Rougher tailing pH |
|----------|---------------|-------------------------|--------------------------|--------------|--------------------|
|          |               |                         | Assay                    | Distribution |                    |
| 12.72    | 1.63          | 0.76                    | 30.47                    | 58.63        | 92.66              |
| 1.50     | 2.00          | 0.70                    | 64.77                    | 69.29        | 95.87              |
| 1.63     | 1.63          | 0.75                    | 13.72                    | 53.21        | 85.60              |
| 1.96     | 1.96          | 1.22                    | 20.25                    | 60.18        | 84.95              |
| 3.10     | 1.93          | 0.90                    | 23.16                    | 59.10        | 93.76              |
| 4.40     | 2.20          | 0.77                    | 52.06                    | 65.25        | 73.80              |
| 3.08     | 2.20          | 1.55                    | 26.65                    | 48.46        | 5.7                |
| 5.26     | 2.63          | 2.47                    | 40.71                    | 54.14        | 94.84              |

<sup>1</sup> Cleaned twice.

## 11

It will be apparent that in the case of all of the ores commercially useful results were obtained except with two very refractory Minnesota ores and a Canadian ore, where the grade was slightly below the present specifications for concentrate. In the case of these ores the difficulty was not due to the efficiency of the flotation but because the ore was highly refractory, containing gangue and iron locked together even in very fine sizes.

All of the petroleum sulfonates referred to in the examples under their trade names are typical petroleum sulfonates of the green acid type or, in the case of Example 10, green acid or mahogany acid type, as commercially obtained from the treatment of petroleum lubricating oil fractions with sulfonating agents, such as sulfuric acid, oleum, and the like.

We claim:

1. A method of beneficiating oxidized iron ores by froth flotation which comprises conditioning the ore at high solids with an acid substance, the anion of which is a constituent of an acid having a dissociation constant not less than  $10^{-7}$ , and which does not adversely affect flotation, an unsulfonated oil, and a collector for oxidized iron minerals containing as its major active constituent water soluble petroleum sulfonates of the green acid type obtained in the refining of petroleum lubricating oils, diluting the thus conditioned pulp to froth flotation density, subjecting it to froth flotation to produce a concentrate relatively rich in iron and a tailing relatively poor in iron, the amount of the acid substance being sufficient so that, in the absence of added alkali,

## 12

the pH of the rougher tailing is in the range of 2 to 6.

2. A method of beneficiating oxidized iron ores by froth flotation which comprises conditioning the ore at high solids with sulfuric acid, and unsulfonated oil, and a collector for oxidized iron minerals containing as its major active constituent water soluble petroleum sulfonates of the green acid type obtained in the refining of petroleum lubricating oils, diluting the thus conditioned pulp to froth flotation density, subjecting it to froth flotation to produce a concentrate relatively rich in iron and a tailing relatively poor in iron, the amount of the sulfuric acid being sufficient so that in the absence of added alkali, the pH of the rougher tailings is in the range of 2 to 6.

3. A method according to claim 1 in which the unsulfonated oil is a petroleum hydrocarbon oil.

4. A method according to claim 2 in which the unsulfonated oil is a petroleum hydrocarbon oil.

5. A method according to claim 1 in which the ore pulp is conditioned at high solids with the acid, collector and oil, diluted to flotation pulp density and subjected to froth flotation after substantial neutralization of the acid by means of an alkali.

6. A method according to claim 2 in which the ore pulp is conditioned at high solids with the acid, collector and oil, diluted to flotation pulp density and subjected to froth flotation after substantial neutralization of the acid by means of an alkali.

ROBERT B. BOOTH.  
EARL C. HERKENHOFF.